

# United States Patent Office

2,779,698

Patented Jan. 29, 1957

1

2,779,698

## METHOD OF IMPROVING MACHINABILITY OF STEEL

Robert W. Baughman, Youngstown, Ohio, and Raymond A. Grange, Livingston, N. J., assignors to United States Steel Corporation, a corporation of New Jersey

No Drawing. Application November 4, 1955,  
Serial No. 545,112

10

2 Claims. (Cl. 148—21.5)

This invention relates to a method of improving the machinability of steel and more particularly to improving the machinability of carburizing grades of steel.

Many machine parts, such as gears, are made of low carbon steel containing less than .30% carbon and are carburized to produce a hard wear resistant surface with a tough low carbon core. The parts are ordinarily machined to final size or to approximate size prior to carburizing and afterwards finished to final size by grinding or lapping. Since the finished parts must be quite smooth, the smoothness of the surface following machining is of great importance since it determines the amount of expensive grinding or lapping required to achieve the desired degree of smoothness.

Heretofore it has been common practice to normalize or normalize and temper these steels prior to machining. This frequently causes a "gummy" condition which results in a rough machined surface because the steel is quite soft and is striated, i. e. contains bands of ferrite.

We have discovered that the rough machined surface resulting from the foregoing treatment can be eliminated, and a smooth unpitted surface obtained by treating ferritic steel containing less than .3% carbon, with the balance iron and other elements in amounts which do not adversely affect the properties in the following manner prior to machining. Such steel in the as-rolled or as-forged condition is heated or "austenitized" at a temperature determined by the formula

$$TA = Ae_1 + \frac{2}{3}(Ae_3 - Ae_1)$$

when  $TA$  is the furnace temperature,  $Ae_1$  the lower equilibrium temperature and  $Ae_3$  the upper equilibrium temperature. The material should be held in the furnace until the temperature of the workpiece is equilized throughout at such temperature. By using the temperature derived by the formula, the workpiece will have a structure of about 50% austenite—50% ferrite,  $\pm 10\%$ . This structure is essential since if less austenite than this is formed the final structure will be too soft and machine in a "gummy" fashion; if more austenite than this forms, the final structure will be too hard. After the temperature has been equalized at the  $TA$  holding temperature, the workpiece may be cooled in any convenient way to the bainite formation range, i. e. about 500 to 1000° F. for steels containing up to .3% carbon. The steel must be cooled slowly enough through this range to insure essentially complete transformation to bainite. In some steels, depending on alloy content, an air cool will suffice, in others retarded cooling will be necessary. Such retarded cooling may be accomplished by moving the workpiece to a cooler section of the furnace, moving to a second furnace or by turning the furnace down to about 500° F., i. e. about the  $M_s$  point of the untransformed austenite and permitting the temperature of the workpiece to equalize thereat and hold for any additional time as may be required to complete the transformation to bainite. Thereafter the workpiece may be cooled to room temperature in any convenient manner.

2

In accordance with the foregoing principles, we have treated as rolled 1 1/4 inch diameter bars of SAE 4317 steel containing .15-.20% carbon, .45-.65% manganese, 1.65-2.00% nickel, .40-.60% chromium, .20-.30% molybdenum, with the balance substantially iron. The heating or austenitizing temperature  $TA$  was 1410° F., which was derived in accordance with the formula as follows:

$$\begin{aligned} TA &= Ae_1 + \frac{2}{3}(Ae_3 - Ae_1) \\ &= 1270 + \frac{2}{3}(1480 - 1270) \\ &= 1410^\circ \end{aligned}$$

A sample of the steel so treated was quenched to room temperature and had a microstructure of about 50% ferrite and 50% austenite. Following this, the bars were cooled in the furnace from 1410 to 500° F. and then removed and cooled in air to room temperature. During cooling from 1410 to about 1000° F., about half of the austenite formed at 1410° F. transformed to additional ferrite leaving comparatively small uniformly distributed volumes of austenite. The latter are greatly enriched in carbon by the rejection of ferrite, that is, most of the carbon of the steel is present in the austenite phase. On cooling from 1000 to 500° F. most of the austenite transformed to bainite leaving small, uniformly distributed colonies of bainite. The few small particles of what was either austenite or martensite which remained were too few and too small to appreciably influence machining.

Bars of SAE 4317 steel of the same composition as the foregoing were treated in the conventional way by normalizing from 1700° F. and then tempering at 1200° F. These bars had a severely banded structure and were much rougher after machining.

It was also observed that the bars treated in accordance with this invention had more broken-up chips, especially, on the lighter cuts, and did not become hot indicating that less energy was required. They also sawed in about  $\frac{1}{2}$  less time than the normalized and tempered bar.

While we have described one specific embodiment of our invention, it will be understood that this embodiment is merely for the purpose of illustration and description and that various other forms may be devised within the scope of our invention, as defined in the appended claims.

We claim:

1. A method of improving the machinability of ferritic steels containing less than .3% carbon with the balance iron and other elements in amounts which do not adversely affect the properties, comprising heating said steel at a temperature determined by the formula

$$TA = Ae_1 + \frac{2}{3}(Ae_3 - Ae_1)$$

wherein

$TA$  is the furnace temperature

$Ae_1$  is the lower equilibrium temperature

$Ae_3$  is the upper equilibrium temperature

to partially austenitize it, cooling said steel to the bainite transformation range, cooling through such range at a sufficiently slow rate to insure essentially complete transformation of the austenite to bainite and thereafter cooling to room temperature.

2. A method of improving the machinability of ferritic steels containing less than .3% carbon with the balance iron and other elements in amounts which do not adversely affect the properties, comprising heating said steel at a temperature determined by the formula

$$TA = Ae_1 + \frac{2}{3}(Ae_3 - Ae_1)$$

wherein

70  $TA$  is the furnace temperature

$Ae_1$  is the lower equilibrium temperature

$Ae_3$  is the upper equilibrium temperature

for sufficient time to equalize the temperature of the steel at said Ta temperature to produce a structure therein which is substantially 50% austenite and 50% ferrite, cooling said steel to below about 1000° F. and cooling said steel through its bainite transformation range at a 5 sufficiently slow rate to insure essentially complete transformation of the austenite to bainite and thereafter cooling it to room temperature.

References Cited in the file of this patent

UNITED STATES PATENTS

|           |        |       |               |
|-----------|--------|-------|---------------|
| 2,097,878 | Grabe  | ----- | Nov. 2, 1937  |
| 2,563,672 | Boyce  | ----- | Aug. 7, 1951  |
| 2,664,369 | Kiefer | ----- | Dec. 29, 1953 |

OTHER REFERENCES

Metal Progress, October 1949, pages 504-505.